# EUROPEAN PATENT SPECIFICATION

(11) **EP 4 098 725 B1**
(45) Date of publication and mention of the grant of the patent: **06.05.2026**
(21) Application number: 21775495.1
(22) Date of filing: 22.03.2021
(51) Int. Cl.: C10M 169/04, C10M 169/06, C10N 10/12, C10N 40/04, C10N 50/10, C10M 169/00, C10N 20/02, C10N 30/06

(54) **RESIN LUBRICATION GREASE COMPOSITION**
HARZ-SCHMIERFETTZUSAMMENSETZUNG
COMPOSITION DE GRAISSE LUBRIFIANTE POUR RÉSINE

(30) Priority: 23.03.2020 JP 2020051409
(43) Date of publication of application: 07.12.2022
(73) Proprietor: Kyodo Yushi Co., Ltd., Fujisawa-shi, Kanagawa 251-8588 (JP)
(72) Inventor: SOMA Minami, Fujisawa-shi, Kanagawa 251-8588 (JP); TSUTSUI Daisuke, Fujisawa-shi, Kanagawa 251-8588 (JP); SHIBATA Ryo, Fujisawa-shi, Kanagawa 251-8588 (JP)
(74) Representative: Cabinet Beau de Loménie
(86) International application number: PCT/JP2021/011649
(87) International publication number: WO 2021/193504

(56) References cited:
- EP-A1- 3 239 281
- WO-A1-2009/121378
- WO-A1-2016/155754
- JP-A- 2005 247 971
- JP-A- 2006 044 306
- JP-A- 2006 194 279
- JP-A- 2006 292 083
- JP-A- 2006 292 083
- JP-A- 2007 262 343
- JP-A- 2007 262 344
- JP-A- 2011 512 432
- JP-A- 2017 019 987
- JP-A- 2018 510 947
- JP-A- 2019 116 949
- US-B1- 6 444 621

## Description

### Technical Field

The present invention relates to a use of resin lubrication grease composition, more specifically, a resin lubrication grease composition for lubrication between resin-made members or between a resin-made member and a member made from another material, for example, a metal-made member.

### Background Art

Various metal-made members have conventionally been used as automobile components and the like, but these days, resin-made members are increasingly being used instead of metal-made members for the purpose of reducing the weights. For this reason, both resin-made members and metal-made members are currently used. For example, a resin (polyamide)-made worm wheel gear and a steel-made worm gear are used in a reducer part of electric power steering of automobiles.

As a grease composition to be used for lubrication between resin-made members and between a resin-made member and a metal-made member, Patent Literature 1 describes a lubrication grease composition containing a polyolefin wax. When used for resin lubrication parts, this grease composition can achieve low friction and can meet the demand for improvements in efficiency of components having resin lubrication parts. Patent Literature 2 describes a resin lubrication grease composition characterized in that the grease containing a thickener and a base oil is made contain a montan wax. This grease composition is excellent in that the grease composition can reduce the coefficient of static friction of a lubrication part to extend the durability life of the lubrication part.

However, in the case where these grease compositions are applied to a reducer part of electric power steering, when the steering wheel is slightly turned while the steering is not assisted by a motor, like during the driving on a highway, for example, the lubrication part of the reducer slides, causing a problem that the steering wheel is displaced from the center in some cases, due to the low coefficient of static friction.

### Citation List

### Patent Literatures

Patent Literature 1: Japanese Patent Application Publication No. Hei 9-194867
Patent Literature 2: Japanese Patent Application Publication No. 2002-371290

Each of US 6 444 621 B1, WO 2009/121378 A1, WO 2016/155754 A1, and JP 2006 292083 A shows a resin grease composition with a solid organic molybdenum compound.

A grease composition for lubricating resins of EP 3 239 281 A1 contains a base oil, a diurea compound represented by formula (I) as a thickener: R¹ - NHCONH - R² - NHCONH - R³ (I) (wherein R² represents a bivalent aromatic hydrocarbon group having 6 to 15 carbon atoms, and R¹ and R³ each independently represent a straight-chain or branched alkyl group having 8 to 22 carbon atoms), and a chained hydrocarbon polymer.

JP 2006 194279 A shows a low noise reduction gear provided with a drive gear and a driven gear, each supported by a bearing, and a lubricant composition which includes lubricant and shock absorbing material particles of average particle diameter D1 of 50µm< D1 ≤300µm.

### Summary of Invention

### Problems to be solved by the invention

Therefore, an object of the present invention is to provide a lubrication that can increase the coefficient of static friction of a lubrication part, and suppress an increase in the coefficient of dynamic friction associated with the increased coefficient of static friction and maintain the coefficient of dynamic friction at a certain low level, thus suppressing sliding of the lubrication part of a reducer when no assistance is provided by a motor and maintaining a lubrication efficiency when assistance is provided by the motor.

### Means for solution of the problems

The present invention is defined in the claims.

### Advantageous Effects of Invention

The present invention makes it possible to provide a resin lubrication that can increase the coefficient of static friction of a lubrication part and maintain the coefficient of dynamic friction at a certain low level, thus suppressing sliding of the lubrication part of the reducer when no assistance is provided by a motor and maintaining the lubrication efficiency when assistance is provided by the motor.

### Description of Embodiments

### [Thickener]

The thickener to be used in the grease composition used in the present invention includes a lithium soap thickener. Lithium soap thickeners are e.g. represented by a Li soap and a Li complex soap, urea thickeners represented by diurea, inorganic thickeners represented by organoclay and silica, and organic thickeners represented by PTFE. Since soap thickeners themselves have low coefficients of dynamic friction, an excellent lubrication efficiency can be achieved by using a soap thickener. Lithium 12-hydroxystearate, lithium stearate, and a Li complex soap (for example, a Li complex soap formed from 12-hydroxystearic acid and azelaic acid) are more preferable, and lithium 12-hydroxystearate and a Li complex soap are particularly preferable. Since thickening can be made with a small amount of the thickener by using lithium 12-hydroxystearate and a Li complex soap, an excellent low-temperature operability can be achieved.

The amount of the thickener in the grease composition used in the present invention is 4 to 17% by mass, and preferably 5 to 15% by mass based on the total mass of the composition. By setting the amount to 3% by mass or more, it is possible to achieve a thickener effect sufficient for forming a grease, and to suppress leakage of the grease from lubrication parts. By setting the amount to 20% by mass or less, it is possible to provide the grease composition with a hardness appropriate to flow into lubrication parts.

### [Base Oil]

The base oil to be used in the grease composition used in the present invention may contain mineral oils and/or ester synthetic oils, e.g. represented by diester and polyolester, and contains synthesized hydrocarbon oils, e.g. represented by poly-α-olefin ("PAO"), co-oligomer of ethylene and α-olefin, and polybutene. Two or more of these may be used in combination.

Meanwhile, since the electric power steering has a smaller output than hydraulic power steering, the operation torque of the electric power steering at a low temperature is large, and operation failure sometimes occurs. In the case of using the grease composition used in the present invention for a lubrication part of electric power steering, for example, a reducer part, when a synthetic oil is contained as the base oil, it is possible to reduce the operation torque at a low temperature. Particularly, a synthesized hydrocarbon oil is preferably contained, and poly α-olefin is more preferably contained. The proportion of the synthetic oil in the base oil is not particularly limited, but the proportion of PAO may be set to preferably 50 to 100% by mass, more preferably 60 to 100% by mass, and further preferably 70 to 100% by mass in order to achieve a favorable low-temperature operability. In this case, the type of the balance of the base oil is not a matter, but a mineral oil is preferable from the viewpoint of costs. Hence, in the case of using the grease composition used in the present invention for a lubrication part of electric power steering, for example, a reducer part, the proportion of the mineral oil in the base oil is preferably 0 to 50% by mass, more preferably 0 to 40% by mass (for example, 20 to 40% by mass), and further preferably 0 to 30% by mass. As the mineral oil, any mineral oil can be used. The mineral oil includes, for example, refined mineral oils, high viscosity index oils, and dewaxed mineral oils. Dewaxed mineral oils are particularly preferable from the viewpoint of low-temperature operability.

The kinematic viscosity of the base oil at 40°C is preferably 20 to 80 mm²/s, and more preferably 30 to 70 mm²/s, from the viewpoint of low-temperature operability and durability.

It is particularly preferable that the base oil contain 70 to 100% by mass of PAO having a kinematic viscosity at 40°C of 15 to 420 mm²/s based on the total amount of the base oil. This makes it possible to obtain a grease composition particularly excellent in low-temperature operability. **In** this case, the kinematic viscosity at 40°C of the entire base oil is preferably 30 to 70 mm²/s.

The content of the base oil in the grease composition used in the present invention is an amount that is normally used for production of greases, and is, for example, 75 to 95% by mass, and is preferably 83 to 96% by mass, and more preferably 85 to 95% by mass, from the viewpoint of low-temperature operability.

### [Additive]

Organic molybdenum compounds used as additives for greases in general include those which are solid and liquid at ordinary temperature and ordinary pressure. Since a solid organic molybdenum compound keeps the solid state even when blended in grease, the solid organic molybdenum compound can exhibit a different performance from a liquid organic molybdenum compound.

The solid organic molybdenum compound to be used in the present invention is not particularly limited as long as the solid organic molybdenum compound is solid at ambient temperature (for example, 25°C).

The amount of the solid organic molybdenum compound in the composition used in the present invention is more than 0.5% by mass and less than 7.5% by mass, and is preferably 1 to 5% by mass, and further preferably 2 to 3% by mass. When the amount is more than 0.5% by mass, the coefficient of static friction can be significantly increased, making it possible to suppress sliding of lubricated members. When the amount is less than 7.5% by mass, favorable low-temperature operability and lubrication efficiency of lubricated members can be maintained.

Various additives may be added to the grease composition used in the present invention as necessary. Such additives include, for example, antioxidants, rust inhibitors, metal corrosion inhibitors, oiliness improvers, anti-wear agents, extreme pressure agents, solid lubricants. and the like. Specifically, the antioxidants include amine-based, phenol-based, quinoline-based, sulfur-based antioxidants, zinc dithiophosphates, and the like, and amine-based antioxidants are preferable. The amine-based antioxidants include, for example, phenyl α-naphthylamine, alkylphenyl α-naphthylamine, alkyl diphenylamine, and the like, and alkyl diphenylamine is particularly more preferable.

The rust inhibitors include zinc-based, carboxylic acid-based, carboxylate-based, amine-based, and sulfonate-based rust inhibitors, but sulfonic acid salt-based rust inhibitors, particularly Ca sulfonates, are preferable. The Ca sulfonates include calcium salts of petroleum sulfonic acid obtained by sulfonation of aromatic hydrocarbon components in lubricant oil distillates, calcium salts of synthetic sulfonic acids such as dinonylnaphthalenesulfonic acid and alkyl benzenesulfonic acids, overbased calcium salts of petroleum sulfonic acids, overbased calcium salts of alkyl aromatic sulfonic acids, and the like, and overbased Ca sulfonate is particularly preferable.

The metal corrosion inhibitors include thiadiazole-based, benzimidazole-based, and benzotriazole-based metal corrosion inhibitors, but benzotriazole-based metal corrosion inhibitors are preferable. The benzotriazole-based inhibitors include 1,2,3-benzotriazole, 1,H-benzotriazole, 4-methyl-1,H-benzotriazole, 4-carboxy-1,H-benzotriazole, sodium tolyltriazole, 5-methyl-1,H-benzotriazole, benzotriazole butyl ether, silver benzotriazole, 5-chloro-1,H-benzotriazole, 1-chloro-benzotriazole, 1-di(C8H17)aminomethyl-benzotriazole, 2,3-dihydroxypropyl-benzotriazole, 1,2-dicarboxyethyl-benzotriazole, (C8H17)aminomethyl-benzotriazole, bis(benzotriazole-1-yl-methyl) (C8H17)amine, N,N-bis(2-ethylhexyl)-4-methyl-1H-benzotriazole-1-methyl amine, N,N-bis(2-ethylhexyl)-5-methyl-1H-benzotriazole-1-methylamine, and the like, and 1-[N,N-bis(2-ethylhexyl)aminomethyl]-4-methylbenzotriazole is particularly preferable.

The oiliness improvers include fatty acids, fatty acid esters, and phosphoric acid esters.

The anti-wear agents and the extreme pressure agents include phosphorus-based, sulfur-based, and organic metal-based agents.

The solid lubricants include oxidized metallic salts, molybdenum disulfide, polytetrafluoroethylene, melamine cyanurate, and graphite.

The content of these optional additives is, for example, 0.1 to 10% by mass, preferably 0.1 to 5% by mass, and more preferably 0.5 to 3% by mass, based on the total mass of the composition used in the present invention.

The 60-stroke worked penetration of the grease composition used in the present invention is preferably 190 to 415, and more preferably 235 to 370, from the viewpoint of oil release, leakage prevention, and low-temperature operability.

The grease composition used in the present invention can be easily produced by mixing the above components and other additives in a desired blending ratio in accordance with a conventional method.

The grease composition used in the present invention is used for lubrication between resin-made members or between a resin-made member and a member made from another material, for example, a metal-made member. Specifically, the grease composition used in the present invention can be favorably used for rolling-element bearings, ball screws, reducers of electric power steering devices, support yokes, and/or the like. The resin contained in resin-made members is not particularly limited, but a polyamide is preferable from the viewpoint of strength and hardness.

### Examples

### <Test Grease>

### [Test Grease Composition Containing Lithium 12-Hydroxystearate as a Thickener]

First, 570.0 g of 12-hydroxystearic acid was completely dissolved in 2352.3 g of a base oil at 90°C. In a different container, 77.7 g of lithium hydroxide was completely dissolved in 388.5 g of pure water at 90°C, and both were mixed while the temperature was increased to 220°C, and thereafter the mixture was cooled to 100°C or less while agitating, and the resultant was used as a base grease (the total amount of the base grease was 3000 g, the amount of the thickener was 19%).

A solid organic molybdenum compound was blended with the above base grease in the proportion shown in Table 1, and an additional base oil was added such that the proportion of the thickener became the amount shown in Table 1, followed by dispersion using a three roll mill to prepare a test grease composition. The consistency of the test grease composition was 325.

### [Test Grease Composition Containing Lithium Stearate as a Thickener]

First, 957.2 g of stearic acid and 151.3 g of lithium hydroxide monohydrate were added to 1891.5 g of the base oil while agitating, and thereafter the mixture was heated to 230°C. Thereafter, the mixture was cooled to 100°C or less while agitating to obtain a base grease. A solid organic molybdenum compound was blended with the above base grease in the proportion shown in Table 1, and an additional base oil was added such that the proportion of the thickener became the amount shown in Table 1, followed by dispersion using the three roll mill to prepare a test grease composition. The consistency of the test grease composition was 325.

### [Test Grease Composition Containing Lithium Complex Soap as a Thickener]

First, 445.9 g of 12-hydroxystearic acid was added to 1776.0 g of the base oil, and the solution was heated to a temperature (80 to 90°C) at which the solution was turned into a completely transparent liquid state. To this, what was obtained by adding, heating and dissolving 64.8 g of lithium hydroxide monohydrate into 363.5 g of water in advance was added. Then, saponification reaction of 12-hydroxystearic acid was conducted while vigorously agitating to form a lithium salt of 12-hydroxystearic acid. Next, 507.7 g of the base oil and 139.4 g of azelaic acid were added, followed by continuously agitating to obtain a uniform state. To this, what was obtained by adding, heating, and dissolving 64.8 g of lithium hydroxide monohydrate into 363.5 g of water in advance was added, and saponification reaction of azelaic acid was conducted while vigorously agitating. Next, the processing was advanced to a heating step, where the content was gradually heated to 200°C. Thereafter, the content was cooled to 100°C or less while agitating to obtain a base grease. A solid organic molybdenum compound was blended with the above base grease in the proportion shown in Table 1, and an additional base oil was added such that the proportion of the thickener became the amount shown in Table 1, followed by dispersion using the three roll mill to prepare a test grease composition. The consistency of the test grease composition was 325.

The components used to prepare the test grease compositions are as follows:

### <Base Oil>

- PAO: Poly-α-olefin, the kinematic viscosity at 40°C: 56 mm²/s
- Mineral Oil: Naphthene-based mineral oil, the kinematic viscosity at 40°C: 115 mm²/s

Note that the kinematic viscosity were measured in accordance with JIS K 2220 23.

### <Additives>

- Solid organic Mo: MoDTC (Trade name of Molyvan A, produced by R.T.Vanderbilt Company Inc.)
- Polyolefin wax: Polyethylene wax (Trade name: LICOWAX PE190 P, produced by Clariant Chemicals)
- Montan wax: Partially saponified montanic acid ester wax (Trade name: LICOWAX OP FL, produced by Clariant Chemicals)

Note that mass% shown in Table 1 is a value based on the total mass of the grease composition, and the balance is the base oil.

The worked penetration of the test grease composition means the 60-stroke worked penetration and was measured in accordance with JIS K 2220 7.

### <Test Method>

On the grease compositions of Examples and Comparative Examples, a test as described below was conducted, and the arithmetic means of coefficient of friction after stabilization was measured to evaluate the properties of these. The results are shown in Table 1.
∘ Coefficient of Static Friction and Coefficient of Dynamic Friction (Bowden test)

### [Test Conditions]

Test piece: a resin pin (diameter 5.0 mm, length 15 mm, nylon GF30%)
   Plate (2.0×15×160 mm, surface roughness Ra=0.2 µm, S45C)
Sliding velocity: 1 mm/s
Stroke: 10 mm
Load: 19.6 N
Temperature: 25°C
Amount of grease applied: 0.2-mm thickness
Determination criteria: coefficient of static friction
   0.155 or more=o (Passed), less than 0.155=× (Failed)
Determination criteria: coefficient of dynamic friction
   0.150 or less=∘ (Passed), more than 0.150=× (Failed)

## Claims

1. Use of a grease composition in lubrication between a resin-made member and a resin-made member or lubrication between a resin-made member and a member made from another material, wherein
the resin-made member to be lubricated is of a polyamide and said grease composition comprises:
a solid organic molybdenum compound in an amount of more than 0.5% by mass and less than 7.5% by mass relative to a total mass of the composition,
4 to 17% by mass relative to a total mass of the composition of a thickener which includes a lithium soap thickener, and
a synthesized hydrocarbon oil as a base oil.

2. The use according to claim 1, wherein
the content of the solid organic molybdenum compound is 1 to 5% by mass.

3. The use according to claim 1 or 2, wherein
the thickener is lithium stearate, lithium 12-hydroxystearate, or lithium complex soap.

4. The use according to any one of claims 1 to 3, wherein
the base oil of the grease composition further contains a mineral oil.

5. The use according to claim 4, wherein
the proportion of the mineral oil in the base oil is 20 to 50% by mass.

6. The use according to any one of claims 1 to 5, wherein
the member made from another material other than the resin-made member to be lubricated is a metal-made member.

7. The use according to any one of claims 1 to 6, wherein
the thickener consists of the lithium soap thickener as a sole thickener.

8. A reducer for an electric power steering, including a member made of resin together with a further member made of either resin or another material and filled with a grease composition,
**characterized in that**
the grease composition is the one used according to any one of claims 1 to 7 and is filled to provide lubrication between said member and said further member.

## Patentansprüche

1. Verwendung einer Fettzusammensetzung zur Schmierung zwischen einem aus Harz gefertigten Element und einem aus Harz gefertigten Element oder zur Schmierung zwischen einem aus Harz gefertigten Element und einem aus einem anderen Material gefertigten Element, wobei
das zu schmierende aus Harz gefertigte Element aus einem Polyamid ist und die Fettzusammensetzung Folgendes umfasst:
eine feste organische Molybdänverbindung in einer Menge von mehr als 0,5 Massen-% und weniger als 7,5 Massen-%, bezogen auf die Gesamtmasse der Zusammensetzung,
4 bis 17 Massen-%, bezogen auf die Gesamtmasse der Zusammensetzung, eines Verdickungsmittels, das ein Lithiumseifen-Verdickungsmittel beinhaltet, und
ein synthetisiertes Kohlenwasserstofföl als Basisöl.

2. Verwendung nach Anspruch 1, wobei
der Gehalt an der festen organischen Molybdänverbindung 1 bis 5 Massen-% ist.

3. Verwendung nach Anspruch 1 oder 2, wobei
das Verdickungsmittel Lithiumstearat, Lithium-12-hydroxystearat oder Lithiumkomplexseife ist.

4. Verwendung nach einem der Ansprüche 1 bis 3, wobei
das Basisöl der Schmierfettzusammensetzung ferner ein Mineralöl enthält.

5. Verwendung nach Anspruch 4, wobei
der Anteil des Mineralöls an dem Basisöl 20 bis 50 Massen-% ist.

6. Verwendung nach einem der Ansprüche 1 bis 5, wobei
das Element, das aus einem anderen Material gefertigt ist, als das zu schmierende aus Harz gefertigte Element ein aus Metall gefertigtes Element ist.

7. Verwendung nach einem der Ansprüche 1 bis 6, wobei
das Verdickungsmittel aus dem Lithiumseifen-Verdickungsmittel als einzigem Verdickungsmittel besteht.

8. Untersetzungsgetriebe für eine elektrische Lenkung, umfassend ein aus Harz gefertigtes Element zusammen mit einem weiteren Element, das entweder aus Harz oder einem anderen Material gefertigt und mit einer Fettzusammensetzung gefüllt ist,
**dadurch gekennzeichnet, dass**
die Fettzusammensetzung jene ist, die nach einem der Ansprüche 1 bis 7 verwendet wird, und gefüllt ist, um Schmierung zwischen dem Element und dem weiteren Element bereitzustellen.

## Revendications

1. Utilisation d'une composition de graisse pour la lubrification entre un élément fabriqué à base de résine et un élément fabriqué à base de résine ou pour la lubrification entre un élément fabriqué à base de résine et un élément fabriqué à base d'un autre matériau, dans laquelle
l'élément fabriqué à base de résine à lubrifier est d'un polyamide et ladite composition de graisse comprend :
un composé organique solide de molybdène en une quantité supérieure à 0,5 % en poids et inférieure à 7,5 % en poids par rapport au poids total de la composition,
de 4 à 17 % en poids par rapport au poids total de la composition d'un épaississant qui comprend un épaississant de savon de lithium, et
une huile hydrocarbonée synthétisée en tant qu'huile de base.

2. Utilisation selon la revendication 1, dans laquelle
la teneur en composé organique solide de molybdène est de 1 à 5 % en poids.

3. Utilisation selon la revendication 1 ou 2, dans laquelle
l'épaississant est le stéarate de lithium, le 12-hydroxystéarate de lithium, ou un savon complexe de lithium.

4. Utilisation selon l'une quelconque des revendications 1 à 3, dans laquelle
l'huile de base de la composition contient en outre une huile minérale.

5. Utilisation selon la revendication 4, dans laquelle
la proportion de l'huile minérale dans l'huile de base est de 20 à 50 % en poids.

6. Utilisation selon l'une quelconque des revendications 1 à 5, dans laquelle
l'élément fabriqué à base d'un autre matériau autre que l'élément fabriqué à base de résine à lubrifier est un élément fabriqué à base de métal.

7. Utilisation selon l'une quelconque des revendications 1 à 6, dans laquelle
l'épaississant se compose de l'épaississant de savon de lithium en tant qu'unique épaississant.

8. Réducteur pour direction assistée électrique, comprenant un élément en résine conjointement avec un autre élément en résine ou en autre matériau et rempli avec une composition de graisse,
**caractérisé en ce que**
la composition de graisse est celle utilisée selon l'une quelconque des revendications 1 à 7 et est remplie pour fournir une lubrification entre ledit élément et ledit autre élément.
